

May 17, 1966

R. F. CRAIG ET AL

3,251,598

PLASTIC COMPOSITION AND BOWLING PIN MADE THEREOF

Filed March 13, 1961



INVENTORS

R. F. CRAIG  
R. J. MARTINOVICH

BY

*Hudson E. Young*

ATTORNEYS

1

3,251,598

**PLASTIC COMPOSITION AND BOWLING PIN  
MADE THEREOF**

Robert F. Craig and Robert J. Martinovich, Bartlesville, Okla., assignors to Phillips Petroleum Company, a corporation of Delaware

Filed Mar. 13, 1961, Ser. No. 95,091  
11 Claims. (Cl. 273—82)

This invention relates to a novel plastic composition and an article of manufacture made thereof, namely a bowling pin.

In the last decade or so there has been a rapid increase in the number of bowling establishments in this country due to the widespread public interest and participation in the sport of bowling. Along with this there have been proposed, patented, and evaluated a number of different materials as substitutes for some or all of the wood now generally used in bowling pins in an attempt to satisfy the demand for a more durable, cheap, and useful bowling pin having a longer life.

At the present time, all bowling pins approved by the American Bowling Congress are constructed of hard maple, some of which are coated with lacquer or a thin layer of plastic. While these wooden bowling pins have enjoyed long and widespread use, they do have a number of shortcomings. The scorability of these hard maple bowling pins is not uniform, but rather varies over the useful life of the pin; new pins (i.e., less than 300 lines) have low scorability, and as the pins get older this scorability tends to increase. In order to obtain maximum pin life for such wooden bowling pins it is common to "rest" the pins by taking them out of service after every 300-500 lines of service, during which time the wood fibers reform to a degree and enable the bowling lane proprietor to refinish those pins which are worn, chipped, marred, splintered, or otherwise damaged. The useful life of the average wooden pin is only about 2500 to 3500 lines. Another disadvantage in the use of bowling pins made of hard maple is that there is a shortage of select hard maple, and it is necessary to grade the wooden pins because of variations in the character of the hard maple that is used in making the pins. Moreover, such variation in the wood means that the densities of the pins made from various grades of hard maple will vary.

To date none of the materials proposed or evaluated as substitutes for the hard maple of the bowling pins has been able to meet the rigid specifications and standards of the American Bowling Congress and gain acceptance. In particular, all-plastic bowling pins made from plastics such as cellulose acetate, cellulose acetate butyrate, styrene, and conventional (low density) polyethylene have been rejected as substitutes because they have proven to be unsatisfactory for a number of reasons; for example, such plastics have proven to be too brittle, too hard, and some materials cannot be readily and economically fabricated or machined, while others have not been sufficiently durable and have not been able to withstand the harsh treatment encountered in automatic pin setting equipment and upon repeated impact by bowling balls.

Accordingly, an object of this invention is to provide a novel plastic composition. Another object is to provide as a new article of manufacture a bowling pin made of a novel plastic composition, the properties of which make it ideally suited for the fabrication of bowling pins therefrom. Another object is to provide a bowling pin made of a novel plastic composition, which bowling pin is durable, has a relatively long useful life, has a high and uniform scorability, a desirable coefficient of friction, and high impact strength, and other properties which make it especially suitable as a substitute for the hard

2

maple of bowling pins now generally used. Other objects and advantages of this invention will become apparent to those skilled in the art from the following discussion, appended claims, and accompanying drawing which illustrates in the single figure an elevational view in half-section of a preferred embodiment of the improved bowling pin of this invention.

The novel plastic composition of this invention, which is especially suited in fabricating an improved bowling pin, broadly comprises about 80 to 90 weight percent of a copolymer of ethylene and 1-butene having a melt index (hereinafter defined) of 0.3 to 1.2 and about 20 to 10 weight percent of an isobutylene polymer such as polyisobutylene or, preferably, a copolymer of isobutylene and a conjugated diene such as isoprene or 1,3-butadiene. As will be established in detail by the examples of this specification, bowling pins made from said novel plastic composition have uniform scorability throughout the life of the pin, and said pins have a useful life which is far greater than that of wooden pins made of hard maple. Further, the bowling pins of this invention have a greater ability to withstand impact, require a minimum of maintenance, they can be fabricated in an efficient and economical manner, and their use eliminates the grading and sale of "odd lot" pins fabricated from hard maple.

The copolymer of ethylene and 1-butene used in accordance with this invention has a density (hereinafter defined) of from 0.948 to 0.952; this represents an incorporation of from 1.5 to 1.0 weight percent, respectively, based on total monomers, of the 1-butene comonomer into the copolymer molecule. Preferably, the density of the copolymer is approximately 0.950 to 0.951. The melt index of these copolymers is in the range of approximately 0.3 to 1.2. Copolymers of this type are preferably prepared by the copolymerization of a major amount of ethylene and a minor amount of 1-butene in the presence of a catalyst consisting essentially of chromium oxide supported on a silica-alumina composite, the catalyst containing at least 0.1 weight percent chromium in the hexavalent state. The total chromium content of the catalyst is generally, though not necessarily, within the range of 1 to 10 weight percent of the total catalyst. The copolymerization is frequently carried out at a temperature within the range of from about 230 to 300° F. Ordinarily, the copolymerization is conducted in the presence of a hydrocarbon diluent which is liquid and inert under the reaction conditions. Generally, this diluent is a naphthene or a paraffin hydrocarbon having from 3 to 12 carbon atoms per molecule. Examples of such hydrocarbons are normal pentane, normal hexane, 2,2,4-trimethylpentane, cyclohexane and methylcyclopentane. The catalyst is preferably used as a granular suspension thereof in the diluent. Further details of this process can be obtained by a reading of U.S. Patent 2,825,721 which was issued March 4, 1958, to J. P. Hogan and R. L. Banks. Other suitable copolymers, though less preferred than those already described herein, can be obtained by the copolymerization of ethylene and 1-butene at approximately the temperatures already described herein, in the presence of a catalyst prepared from or containing organometal compounds. Examples of such catalysts are those obtained by mixing, for example, triethylaluminum with titanium tetrachloride, a mixture of diethylaluminum monochloride and monoethylaluminum dichloride with titanium tetrachloride, a mixture of ethylaluminum chloride with titanium tetrabutoxide, and similar catalysts, discussed in more detail in U.S. Patent 2,846,427, issued August 5, 1958, to R. A. Findlay, and U.S. Patent 2,826,447, issued March 18, 1958, to Gene Nowlin and H. D. Lyons.

A number of copolymer of ethylene and 1-butene, made in the manner described, which are useful in the

practice of this invention are set forth in Table I together with certain physical properties.

The density referred to herein, is determined by ASTM Method D 1505-57T. Ethanol and water were used as the suspending liquids. The samples used for density determination are prepared by compression-molding molten pellets of the ethylene polymer to form a slab about 6 inches square and  $\frac{1}{2}$  to  $\frac{1}{2}$  inch thick. The slabs are molded at 20,000 p.s.i. and 330° F. The heat is then turned off. Tap water is circulated through the mold cooling system. The slab is cooled to 200° F. at the rate of 25° F. per minute, and then to 150° F. as rapidly as possible by increasing the flow rate of the cooling water. The slab is then removed from the mold and allowed to stand for 24 hours at room temperature. Small pieces of the slab, e.g. about  $\frac{1}{4}$  inch squares, are cut off for the density determination. These pieces are examined to be sure that they have no surface pits or other features which might occlude or entrap air when immersed in liquid.

The melt index, as referred to herein, is determined in accordance with ASTM Method D 1238-52T.

minor amount of the isobutylene polymer. Generally, the amounts of said materials used will be sufficient to provide a blend comprising 80 to 90 weight percent of the ethylene-1-butene copolymer and about 20 to 10 weight percent of the isobutylene polymer. While the plastic composition of this invention can consist essentially of just these two polymeric materials, it is also within the scope of this invention to incorporate in the plastic blend various other materials such as pigments, e.g., titanium dioxide in an amount up to one weight percent of the final blend (preferably about 0.4 weight percent), various anti-static materials for the purpose of preventing the accumulation of dirt, and other materials for special effects.

The plastic composition of this invention can be prepared by placing the desired quantities of the ethylene copolymer and isobutylene polymer (and other ingredients where used) in a Banbury mixer (without prior heating) and mixing the materials in said mixer for a period of time and at a temperature sufficient to obtain a homogeneous blend, e.g., 5 to 7 minutes to a temperature of about 300 to 350° F., preferably about 320° F. The resulting blend-

TABLE I

| Property                                                       | Test            | Ethylene-1-butene copolymer |         |         |
|----------------------------------------------------------------|-----------------|-----------------------------|---------|---------|
|                                                                |                 | A                           | B       | C       |
| Density, gms./cc.                                              | ASTM D 1505-57T | 0.950                       | 0.950   | 0.950   |
| Melt index                                                     | ASTM D 1238-57T | 0.3                         | 0.5     | 1.2     |
| Environmental stress cracking resistance, F <sub>50</sub> hrs. | ASTM D 1693-59T | 350                         | 175     | 55      |
| Tensile strength, 20 in./min., p.s.i.                          | ASTM D 638-58T  | 3,800                       | 3,800   | 3,800   |
| Elongation, 20 in./min., percent                               | ASTM D 638-58T  | 70                          | 50      | 40      |
| Impact strength, ft. lbs./in. notch                            | ASTM D 256-56   | 4.0                         | 2.0     | 1.0     |
| Vicat softening temp., ° F.                                    | ASTM D 1525-58T | 255                         | 255     | 255     |
| Brittleness temp., ° F.                                        | ASTM D 746-57T  | <-180                       | <-180   | <-180   |
| Stiffness, p.s.i.                                              | ASTM D 747-58T  | 115,000                     | 115,000 | 115,000 |
| Hardness                                                       | Shore D         | 67                          | 67      | 67      |

The isobutylene polymer used in conjunction with the afore-described copolymer of ethylene and 1-butene can be polyisobutylene (such as that commercially sold as "Visitanex"). However, we prefer to use a copolymer of isobutylene and a small amount, e.g., 1-2.5 mole percent, of a conjugated diene having 4 to 8 carbons per molecule such as isoprene, butadiene, dimethylbutadiene, piperylene, hexadiene-1,3, and the like. The preparation of these isobutylene polymers by low-temperature catalytic polymerization is well known in the art and need not be described herein in detail. One useful method of preparing polyisobutylene is that disclosed in U.S. Patent 2,240,582. These polyisobutlenes will have varying molecular weights, for example in the range of 1,000 to 1,000,000 and are characterized as rubbery solids which are tough, elastic materials having an elastic memory. These polyisobutlenes and a method of molecular weight determination (Staudinger Viscosity Method) are described in an article by Thomas et al. in "Industrial and Engineering Chemistry," 32, p. 299 (1940). The preparation of the rubbery copolymers of isobutylene and conjugated dienes is also well known, and U.S. Patents 2,356,128, 2,356,129 and 2,356,130 disclose their preparation. These copolymers are known in the art as butyl rubbers. Butyl rubbers with Mooney viscosities of 30 to 80, preferably 60 to 75, can be used in the plastic composition of this invention. A useful commercial product of this type which can be used in this invention is Enjay Butyl 268, which is a copolymer of isobutylene and 1.5 weight percent isoprene having an average mole percent unsaturation of 1.4 and a Mooney viscosity of 71. Other examples of butyl rubber known in the art are "GR-I," "Butyl A," "Butyl C," and "Flexon."

The plastic composition used in making the bowling pins of this invention can be prepared by blending or mixing a major amount of the ethylene-1-butene copolymer and a

minor amount of the isobutylene polymer. Generally, the amounts of said materials used will be sufficient to provide a blend comprising 80 to 90 weight percent of the ethylene-1-butene copolymer and about 20 to 10 weight percent of the isobutylene polymer. While the plastic composition of this invention can consist essentially of just these two polymeric materials, it is also within the scope of this invention to incorporate in the plastic blend various other materials such as pigments, e.g., titanium dioxide in an amount up to one weight percent of the final blend (preferably about 0.4 weight percent), various anti-static materials for the purpose of preventing the accumulation of dirt, and other materials for special effects.

The plastic composition of this invention can be prepared by placing the desired quantities of the ethylene copolymer and isobutylene polymer (and other ingredients where used) in a Banbury mixer (without prior heating) and mixing the materials in said mixer for a period of time and at a temperature sufficient to obtain a homogeneous blend, e.g., 5 to 7 minutes to a temperature of about 300 to 350° F., preferably about 320° F. The resulting blend-

TABLE II

| Property                                                       | Test            | Value  |
|----------------------------------------------------------------|-----------------|--------|
| Density, gms./cc.                                              | ASTM D 1505-57T | 0.948  |
| Melt index                                                     | ASTM D 1238-57T | 0.45   |
| Environmental stress cracking resistance, F <sub>50</sub> hrs. | ASTM D 1693-59T | >480   |
| Tensile strength, 20 in./min., p.s.i.                          | ASTM D 638-58T  | 2,800  |
| Elongation, 20 in./min., percent                               | ASTM D 638-58T  | 160    |
| Impact strength, ft. lbs./in. notch                            | ASTM D 256-56   | 12     |
| Vicat softening temp., ° F.                                    | ASTM D 1525-58T | 244    |
| Brittleness temp., ° F.                                        | ASTM D 746-57T  | -110   |
| Stiffness, p.s.i.                                              | ASTM D 747-58T  | 64,000 |
| Hardness                                                       | Shore D         | 65     |
| Coefficient of friction (kinetic)                              |                 | 0.36   |

The plastic composition of this invention has physical properties which make it especially well-suited for use in the making of bowling pins, such as Shore D hardness values of about 61 to 67 and coefficient of friction (kinetic) values of about 0.36 to 0.40. The coefficient of friction value, as used herein, is that value obtained by placing one compression molded sheet of the plastic composition in a transverse bed between the force exerting members of an Instron electronic tension testing machine, Model No. TCC. A second sheet of the same plastic

composition is attached at one end to a weight or sled of known weight (e.g., 4.3 lbs.) which is affixed to a wire that is passed over a pulley and attached to one of the force exerting (or pulling) members of the testing machine, so as to pull or slide the second sheet of plastic over the first sheet in the stationary bed. The pounds of force (discounting the static friction between the two sheets of plastic) necessary to pull the second sheet over the first sheet, as indicated by the testing machine dial, is determined and this value is divided by the weight of the sled affixed to the second sheet to give the coefficient of friction (kinetic) of the plastic composition.

The accompanying drawing illustrates in its single figure a preferred embodiment of the novel bowling pin of this invention. Referring to that drawing, the bowling pin

Table IV, together with their coefficient of friction and hardness properties.

TABLE III

| 5                                                       | Property        | Test    | Value |
|---------------------------------------------------------|-----------------|---------|-------|
| Density                                                 | ASTM D 1505-57T | 0.950   |       |
| Melt index                                              | ASTM D 1238-57T | 4.0     |       |
| Environmental stress cracking resistance, $F_{50}$ hrs. | ASTM D 1693-59T | 20      |       |
| 10 Tensile strength, 20 in./min. p.s.i.                 | ASTM D 638-58T  | 3,800   |       |
| Elongation, 20 in./min., percent                        | ASTM D 638-58T  | 30      |       |
| Impact strength, ft. lbs./in. notch                     | ASTM D 256-56   | 0.8     |       |
| Vicat softening temp., $^{\circ}$ F                     | ASTM D 1525-58T | 255     |       |
| Brittleness temp., $^{\circ}$ F                         | ASTM D 746-57T  | -160    |       |
| 15 Stiffness, p.s.i.                                    | ASTM D 747-58T  | 115,000 |       |
| Hardness                                                | Shore D         | 67      |       |

TABLE IV

| Type of composition | Ingredients, weight percent             |              |                       | Coefficient of friction, kinetic | Hardness, Shore D |
|---------------------|-----------------------------------------|--------------|-----------------------|----------------------------------|-------------------|
|                     | Ethylene-1-butene copolymer (Table III) | Butyl rubber | Glyceryl tri-stearate |                                  |                   |
| 1                   | 75                                      | 15           | 10                    | 0.442                            | 58-61             |
| 2                   | 80                                      | 15           | 5                     | 0.442                            | 60-63             |
| 3                   | 70                                      | 20           | 10                    | 0.463                            | 57-59             |
| 4                   | 85                                      | 15           | 0                     | 0.400                            | 62-64             |
| 5                   | 80                                      | 10           | 10                    | 0.442                            | 61-62             |
| 6                   | 85                                      | 10           | 5                     | 0.358                            | 62-65             |

comprises an elongated main body 1 with a neck portion defined by the smallest cross sectional area and a ball impact portion defined by the largest cross sectional area, head cap 2, and base cap 3, which elements can be heat sealed by a butt weld at 5 and 6 to form a hollow 7. The pin portions are formed from the novel plastic composition disclosed herein, preferably by injection molding. The pin further comprises a base 8 and base locking pin 9 having suitable key slots 10 therein. The base 8 can be provided with one or more lugs where it abuts the lower end of base cap 3, and locking pin 9 can be turned to 90° to secure this lower pin assembly together. These

30 Pins made of the compositions shown in Table IV upon subjecting the same to bowling alley service were found to have unsatisfactory durability, in that they exhibited excessive neck fracture and, in the case where glyceryl tri-stearate wax was incorporated in the composition, delamination of components, the average life of these pins being less than 3000 lines. All of the compositions used in making these pins are outside the scope of this invention, but serve here for purpose of comparison.

35 Complete sets of regulation size bowling pins were made of the compositions shown in Table V and also subjected to bowling alley service.

TABLE V

| Type of composition | Ingredients, weight percent |              |                       | Coefficient of friction (kinetic) | Hardness, Shore D |
|---------------------|-----------------------------|--------------|-----------------------|-----------------------------------|-------------------|
|                     | Ethylene-1-butene copolymer | Butyl rubber | Glyceryl tri-stearate |                                   |                   |
| 7                   | <sup>1</sup> 85             | 15           | 0                     | 0.400                             | 62-64             |
| 8                   | <sup>2</sup> 85             | 10           | 5                     | 0.358                             | 62-65             |
| 9                   | <sup>2</sup> 85             | 15           | 0                     | 0.400                             | 62-63             |

<sup>1</sup> Table III.

<sup>2</sup> B in Table I.

latter elements 9, 10 can also be formed of the novel plastic composition of this invention or other plastic materials, such as cellulose butyrate. This preferred embodiment has proven to be extremely durable with a pin life in excess of 4300 lines without any fracture and with a high and uniform scorability. It should be understood, of course, that this invention is not to be limited to this embodiment, since this aspect of invention broadly resides in a bowling pin of the plastic composition described without limiting the same to any specific design.

Further objects and advantages of this invention will now be illustrated by the following examples, but it should be understood that the various materials, properties, additives, etc., set forth in these examples should not be construed to limit this invention.

#### Examples

Complete sets of regulation size bowling pins were made of various amounts of ethylene-1-butene copolymer (see Table III for properties) and butyl rubber (Enjay Butyl 268). These bowling pin compositions are shown in

60 Pins made of composition 9 according to this invention were found to be extremely durable with a life in excess of 4300 lines, while pins made of composition 8 (with a low coefficient of friction) exhibited delamination of ingredients, and pins made of composition 7 were not durable because of neck failure and had an average life of less than 2600 lines.

65 In the course of our investigations, we have found that bowling pins made entirely of low pressure (high density) polyethylene homopolymer were not durable in that they exhibited neck failure, e.g., after 350 lines. Other pins made only of the copolymer of ethylene and 1-butene (A in Table I), although durable, were too hard (69-71 Shore D hardness) and had low scorability characteristics.

70 We have also found that pins made of about 70 weight percent of a copolymer of ethylene and 1-butene (B in Table I) and about 30 weight percent polyisobutylene (Vistanex) had a high coefficient of friction (0.632) and low hardness (56-58 Shore D), these pins exhibiting unsatisfactory scorability characteristics.

The above examples establish that bowling pins made of the novel composition disclosed herein are durable, have long life, and desirably high and uniform scorability. Said examples further establish the criticality in blending 80 to 90 weight percent of a copolymer of ethylene and 1-butene, with melt indexes of 0.3 to 1.2, and 20 to 10 percent of a polymer of isobutylene, to provide a blended composition useful in making bowling pins.

Various modifications and alterations of this invention will become apparent to those skilled in the art from the foregoing discussion and accompanying drawing, and it should be understood that this invention is not to be unduly limited to that set forth herein for illustrative purposes.

We claim:

1. A bowling pin comprising an elongated main body, head cap, and base cap elements each molded from a plastic composition comprising about 80 to 90 weight percent of a copolymer of ethylene and 1-butene having a melt index in the range of about 0.3 to 1.2, and about 10 to 20 weight percent of a polymer of isobutylene selected from the group consisting of polyisobutylene and a copolymer of isobutylene and a conjugated diene having 4 to 8 carbon atoms per molecule.

2. A bowling pin comprising an elongated main body, head cap, and base cap elements each molded from a plastic composition comprising about 80 to 90 weight percent of a copolymer of ethylene and 1-butene having a melt index in the range of about 0.3 to 1.2, and about 10 to 20 weight percent of polyisobutylene.

3. A plastic composition comprising about 80 to 90 weight percent of a copolymer of ethylene and 1-butene having a melt index in the range of about 0.3 to 1.2, and about 10 to 20 weight percent of a copolymer of isobutylene and a conjugated diene having 4 to 8 carbon atoms per molecule.

4. A plastic composition comprising about 80 to 90 weight percent of a copolymer of ethylene and 1-butene having a melt index in the range of about 0.3 to 1.2, and about 10 to 20 weight percent of a copolymer of isobutylene and isoprene.

5. A plastic composition comprising about 86 weight percent of a copolymer of ethylene and 1-butene with a melt index of about 0.5, and about 14 weight percent of a copolymer of isobutylene and a conjugated diene having 4 to 8 carbon atoms per molecule, said plastic composition having a Shore D hardness of about 61 to 67 and a coefficient of friction (kinetic) of about 0.36 to 0.40.

6. A plastic composition consisting essentially of about 80 to 90 weight percent of a copolymer of ethylene and 1-butene having a melt index in the range of 0.3 to 1.2 and a density in the range of 0.948 to 0.952, and about 10 to 20 weight percent of a copolymer of isobutylene and isoprene.

7. A bowling pin comprising an elongated main body, head cap, and base cap elements each molded from a plastic composition consisting essentially of about 80 to 90 weight percent of a copolymer of ethylene and 1-butene having a melt index in the range of 0.3 to 1.2 and a density in the range of 0.948 to 0.952, and about 10 to 20 weight percent of a copolymer of isobutylene and isoprene.

8. A plastic composition consisting essentially of about 86 weight percent of a copolymer of ethylene and 1-butene with a melt index of about 0.5 and a density of about 0.948, and about 14 weight percent of a copolymer of isobutylene and about 1.5 weight percent isoprene with an average mole percent unsaturation of about 1.4 and a Mooney viscosity of about 71, said plastic composition

having a Shore D hardness of about 61 to 67 and a coefficient of friction (kinetic) of about 0.36 to 0.40.

9. A bowling pin comprising an elongated main body with a neck portion defined by the smallest cross sectional area and a ball impact portion defined by the largest cross sectional area of said main body, a head cap surmounting said main body, and a base cap depending from said main body, said head cap, main body, and base cap being secured at their adjacent portions to form a hollow, said head cap, main body, and base cap being made of a plastic composition comprising about 80 to 90 weight percent of a copolymer of ethylene and 1-butene having a melt index in the range of about 0.3 to 1.2, and about 10 to 20 weight percent of a polymer of isobutylene selected from the group consisting of polyisobutylene and a copolymer of isobutylene and a conjugated diene having 4 to 8 carbon atoms per molecule.

10. A bowling pin comprising an elongated main body with a neck portion defined by the smallest cross sectional area and a ball impact portion defined by the largest cross sectional area of said main body, a head cap surmounting said main body, and a base cap depending from said main body, said head cap, main body, and base cap being secured at their adjacent portions to form a hollow, said head cap, main body, and base cap being made of a plastic composition comprising about 86 weight percent of a copolymer of ethylene and 1-butene with a melt index of about 0.5, and about 14 weight percent of a copolymer of isobutylene and a conjugated diene having 4 to 8 carbon atoms per molecule.

11. A bowling pin comprising an elongated main body with a neck portion defined by the smallest cross sectional area and a ball impact portion defined by the largest cross sectional area of said main body, a head cap surmounting said main body, and a base cap depending from said main body, said head cap, main body, and base cap being secured at their adjacent portions to form a hollow, said head cap, main body, and base cap being made of a plastic composition consisting essentially of about 86 weight percent of a copolymer of ethylene and 1-butene with a melt index of about 0.5 and a density of about 0.948, and about 14 weight percent of a copolymer of isobutylene and about 1.5 weight percent isoprene with an average mole percent unsaturation of about 1.4 and a Mooney viscosity of about 71.

#### References Cited by the Examiner

##### UNITED STATES PATENTS

|    |           |        |                    |           |
|----|-----------|--------|--------------------|-----------|
| 50 | 2,369,471 | 2/1945 | Latham             | 260—45.5  |
|    | 2,684,504 | 7/1954 | Sell               | 273—82 XR |
|    | 2,791,576 | 5/1957 | Field et al.       | 260—45.5  |
|    | 2,825,721 | 3/1958 | Hogan et al.       | 260—94.9  |
|    | 2,830,919 | 4/1958 | Schatzel           | 260—45.5  |
| 55 | 3,025,061 | 3/1962 | Ernst et al.       |           |
|    | 3,044,777 | 7/1962 | Friedman           | 273—82    |
|    | 3,048,400 | 8/1962 | Friedman           | 273—82    |
|    | 3,074,616 | 1/1963 | Martinovich et al. | 260—89 XR |
| 60 | 3,169,766 | 2/1965 | Ernst              | 273—82    |

##### FOREIGN PATENTS

597,760 5/1960 Canada.

##### OTHER REFERENCES

65 De Coste et al.: Ind. Eng. Chem., vol. 43, pp. 117—121, 1951.

RICHARD C. PINKHAM, Primary Examiner.

LOUIS R. PRINCE, Examiner.